

# United States Patent

## Stuetz

[15] 3,656,903

[45] Apr. 18, 1972

[54] **DIRECT PRODUCTION OF GRAPHITE FIBROUS MATERIALS FROM PREOXIDIZED ACRYLIC FIBROUS MATERIALS**

[72] Inventor: **Dagobert E. Stuetz**, Westfield, N.J.  
[73] Assignee: **Celanese Corporation**, New York, N.Y.  
[22] Filed: **Apr. 10, 1969**  
[21] Appl. No.: **815,200**

[52] U.S. Cl. .... 23/209.1, 23/209.2  
[51] Int. Cl. .... C01b 31/07  
[58] Field of Search. .... 23/209.1; 8/115.5

[56] **References Cited**

UNITED STATES PATENTS

3,281,261 10/1966 Lynch ..... 23/209.1 X  
3,285,696 11/1966 Tsunoda ..... 23/209.1  
3,294,489 12/1966 Millington et al. .... 23/209.1 X  
3,395,970 8/1968 Machell ..... 23/209.4 X  
3,412,062 11/1968 Johnson et al. .... 260/37

3,427,120 2/1969 Shindo et al. .... 23/209.1 X  
3,449,077 6/1969 Stuetz ..... 23/209.1

OTHER PUBLICATIONS

Vosburgh "Textile Research Journal" Vol. 30, 1960, pages 882-896

Primary Examiner—Edward J. Meros  
Attorney—Thomas J. Morgan and C. B. Barris

[57]

ABSTRACT

A rapid process is provided for the direct conversion of a preoxidized acrylic fibrous material containing at least about 7 percent bound oxygen by weight to a fibrous material of predominantly graphitic carbon. The preoxidized acrylic fibrous material is initially impregnated with an organic protective agent and subsequently is passed through a reducing flame which imparts a minimum fiber temperature of at least 1,900°C. while the fibrous material is under tension at least sufficient to prevent visible sagging. In a preferred embodiment of the invention, the reducing flame is generated by a fuel-oxidant mixture, e.g., an acetylene and oxygen mixture.

24 Claims, No Drawings

**DIRECT PRODUCTION OF GRAPHITE FIBROUS MATERIALS FROM PREOXIDIZED ACRYLIC FIBROUS MATERIALS**

**BACKGROUND OF THE INVENTION**

In the search for high performance materials, considerable interest has been focused on graphite fibers. Graphite fibers are defined herein as fibers which consist essentially of carbon and which have a predominant x-ray diffraction pattern characteristic of graphite. Amorphous carbon fibers, on the other hand, are defined as fibers in which the bulk of the fiber weight can be attributed to carbon and which exhibit an essentially amorphous x-ray diffraction pattern. Graphite fibers generally have a much higher modulus and a higher tenacity than do amorphous carbon fibers and in addition are more highly electrically and thermally conductive.

Industrial high performance materials of the future are projected to make substantial utilization of fiber reinforced composites, and graphite fibers theoretically have among the best properties of any fiber, including boron, for use as high strength reinforcement. Among these desirable properties are corrosion and high temperature resistance, low density, high tensile strength, and most important, high modulus. Graphite is one of the very few known materials whose tensile strength increases with temperature. Uses for such graphite-reinforced composites include aerospace structural components, rocket motor casings, deep-submergence vessels and ablative materials for heat shields on reentry vehicles.

One of the major factors retarding the large-scale use of graphite-reinforced composites may be traced to the extreme costs commonly required for the production of high modulus graphite fibers suitable for use as reinforcement. Although the production of fibrous carbon by pyrolysis of hydrocarbon gases has been reported, this technique is generally not suitable for industrial applications requiring good quality control. Graphitization of fibrous organic precursors appears to be the only practical industrial route available to form graphite fibers.

Many of the prior art methods for producing graphite fibers involve long processing periods, high power requirements, and/or expensive and bulky heating apparatus, such as closed furnaces. The processing and equipment costs required to produce graphite fibers commonly dwarf the fiber raw material costs. Often the fiber is of inferior quality due to damage occurring in one or more steps used in its production. For example, amorphous carbon yarn can be converted to graphite yarn by furnace graphitization in a high temperature vacuum oven. In such an oven the hot zone material has commonly been a metal such as tungsten or tantalum. Besides being expensive and slow, this radiant heat method also may result in the deposition of foreign materials such as tungsten, tantalum and/or carbides of these metals on the fiber during the high temperature treatment.

Another prior art approach to graphitizing amorphous carbon fiber, called conductive graphitization, involves passing a yarn over electrically conductive contacts. For example, in one such method an amorphous carbon fiber is advanced over a pair of spaced electrically conductive rollers while passing an electric current through the advancing fiber to raise it to graphitization temperature. A controlled atmosphere of nitrogen, argon, carbon dioxide, or mixtures thereof, generally must be provided around the fiber while undergoing direct resistance heating.

In co-pending U.S. Ser. No. 614,811, filed Feb. 9, 1967 in the names of Dagobert E. Stuetz, Leo R. Belohlav, and Arthur M. Reader, now abandoned, a process is disclosed employing a reducing flame whereby a predominantly amorphous carbonaceous fibrous material containing at least 75 per cent carbon by weight (preferably at least 90 per cent carbon by weight) is converted to a fibrous material of predominantly graphitic carbon. In my co-pending U.S. Ser. No. 615,374, filed Feb. 13, 1967, which issued as U.S. Pat. No. 3,449,077 on June 10, 1969, a process is disclosed whereby a

polybenzimidazole fiber is initially preoxidized and subsequently is passed through a reducing flame where it is graphitized. The above-identified applications are assigned to the same assignee as the instant invention. Heretofore when attempts have been made to directly graphitize a preoxidized acrylic fibrous material by passage through a reducing flame as described hereafter the fibrous configuration has been destroyed. It has accordingly been deemed essential in the past to first carbonize the preoxidized acrylic fibrous material to a carbon content of at least 75 per cent by weight prior to passage through the reducing flame in accordance with the teachings of Ser. No. 614,811.

It is an object of the invention to provide a rapid process for the direct conversion of a preoxidized acrylic fibrous material to a predominantly graphitic fibrous material.

It is an object of the invention to provide a process capable of producing a graphite fiber exhibiting relatively uniform properties.

It is another object of the invention to provide a graphitization process which does not require bulky and highly expensive equipment.

These and other objects, as well as the scope, nature and utilization of the invention will be apparent from the following detailed description and appended claims.

**SUMMARY OF THE INVENTION**

It has been found that a process for producing a predominantly graphitic fibrous material from a preoxidized acrylic fibrous material derived from a fibrous precursor consisting primarily of recurring acrylonitrile units, with said preoxidized acrylic fibrous material having

- a. a carbon content of up to about 65 per cent by weight,
- b. a relatively amorphous x-ray diffraction pattern,
- c. a bound oxygen content of at least about 7 per cent by weight, and
- d. an absence of structural integrity when heated for two seconds at a fiber temperature of 1,900° C., comprises: impregnating the preoxidized acrylic fibrous material with a quantity of an organic protective agent capable of rendering the material resistant to loss of structural integrity when heated for at least two seconds at a fiber temperature of 1,900° C., and passing the impregnated fibrous material through a reducing flame imparting to the material a minimum temperature of at least 1,900° C. at a speed sufficient to avoid breaking while the material is under a tension at least sufficient to prevent visible sagging.

The resulting graphite fibers are suitable for use as a reinforcing medium in composite articles which find particular utility in applications where a strong, lightweight, structural element is required.

**DETAILED DESCRIPTION OF THE INVENTION**

The preoxidized acrylic fibrous material which is graphitized in accordance with the present process has (1) a carbon content of up to about 65 per cent by weight, (2) a relatively amorphous x-ray diffraction pattern, (3) a bound oxygen content of at least 7 per cent by weight, and (4) an absence of structural integrity when heated for two seconds at a fiber temperature of 1,900° C.

The carbon content of the preoxidized acrylic fibrous material will vary with the extent of the preoxidation treatment referred to hereafter, and will commonly range from about 50 to 65 per cent by weight. As the extent of preoxidation increases, the carbon content of the preoxidized fiber commonly tends to decrease. Since the preoxidation treatment is conducted at a moderate temperature, the preoxidized acrylic fibrous material will exhibit a relatively amorphous x-ray diffraction pattern and an absence of an x-ray diffraction pattern characteristic of graphitic carbon.

The bound oxygen content of the preoxidized acrylic fibrous material is at least about 7 per cent by weight as determinable by routine analytical techniques, such as the Unter-

zaucher analysis. A preoxidized acrylic fibrous material suitable for use in the process commonly has a bound oxygen content of about 7 to 15 per cent by weight. Preoxidized acrylic fibrous materials having higher bound oxygen contents tend to require more extended residence times for their production and tend to yield no commensurate advantage in the instant graphitization process.

In the absence of the impregnation treatment described hereafter the preoxidized acrylic fibrous materials utilized in the process lose their structural integrity when heated for two seconds at a fiber temperature of 1,900° C. produced by a reducing flame as described hereafter. Such failure of structural integrity is commonly exhibited by breakage of the fibrous material and partial or complete disintegration. The preoxidized acrylic fibrous materials are commonly non-burning when subjected to an ordinary match flame even in the absence of the impregnation treatment.

The acrylic fibrous precursor from which the preoxidized acrylic fibrous material utilized in the process is derived consists primarily of recurring acrylonitrile units. For instance, the acrylic fibrous precursor should generally contain at least about 85 mol per cent of acrylonitrile units and up to about 15 mol per cent of one or more monovinyl units copolymerized therewith, such as styrene, methyl acrylate, methyl methacrylate, vinyl acetate, vinyl chloride, vinylidene chloride, vinyl pyridine, and the like. In a particularly preferred embodiment of the invention the preoxidized acrylic fibrous material is derived from an acrylonitrile homopolymer.

The preoxidized acrylic fibrous material is formed by the thermal treatment of the fibrous precursor at a relatively moderate temperature in an oxygen-containing atmosphere. The preoxidation treatment may be conducted on either a batch or a continuous basis in accordance with procedures known in the art. U.S. Ser. Nos. 749,957, filed Aug. 5, 1968 of Dagobert E. Stuetz; 749,959, filed Aug. 5, 1968 of Michael J. Ram; and 750,018, filed Aug. 5, 1968 of Michael J. Ram and Richard N. Rulison disclose preferred preoxidation procedures. Each of the above-identified applications is assigned to the same assignee as the instant invention and is herein incorporated by reference. Other preoxidation procedures capable of producing the requisite starting material for use in the instant process may be chosen as will be apparent to those skilled in the art.

The preoxidized acrylic fibrous materials which are graphitized in accordance with the present invention are preferably in yarn form. Appreciable lengths of a continuous multifilament yarn are graphitized in a particularly preferred embodiment of the invention. Staple yarns may also be selected, however, these generally give correspondingly lower tensile properties than do the continuous filament yarns. Other fibrous assemblages, such as fabrics, may likewise be treated in accordance with the present invention as will be apparent to those skilled in the art. When a yarn is selected as the starting material, it may optionally be provided with a twist which improves its handling characteristics. For example, a twist of about 0.1 to 1 tpi, and preferably about 0.1 to 0.7 tpi may be conveniently utilized.

The preoxidized acrylic fibrous material is impregnated prior to subjecting to the reducing flame with an organic protective agent which is capable of rendering the fibrous material resistant to loss of structural integrity when heated in a reducing flame for at least two seconds at a fiber temperature of 1,900° C. As pointed out hereafter, the impregnation step of the process may be conducted on either a batch basis or on a continuous basis.

The organic protective agent may be selected from the group consisting of organic phosphorus compounds, organic antimony compounds, organic tin compounds, halogenated alcohols, halogenated esters, halogenated organic acids, halogenated organic anhydrides, halogenated phenolic compounds, halogenated aliphatic hydrocarbons, halogenated aromatic hydrocarbons, halogenated aromatic ethers, silicon oils, and mixtures of the foregoing.

A variety of organic phosphorus compounds may be selected for use in the process. For instance, organophosphorus compounds such as phosphates, phosphoramides, phosphites, phosphonates, etc. may be utilized. Examples of particular organic phosphates which may be used are tris[2,3-dibromopropyl] phosphate available commercially under the designation "Firemaster T23P" from the Michigan Chemical Corporation, tris[beta-chloroethyl] phosphate, and tricresyl phosphate. Examples of particular phosphoramides which may be used are cyanoethyl bis[dimethyl amino] phosphate and aziridinyl phosphine oxide. Examples of particular phosphites which may be used are triphenylphosphite, and condensation products of triphenylphosphite with bisphenol A (para, para'-isopropylidenediphenol) and pentaerythritol. Examples of particular phosphonates which may be used are monochloromethylphosphonate, and dimethyl[trichloro alpha-hydroxyethyl] phosphonate. Phosphite-phosphonates sold under the designation of "Phosgard" by the Monsanto Company may be selected. Diphosphonium halides such as ethylene bis[tricyanoethyl] phosphonium bromide, tetrakis[hydroxymethyl] phosphonium chloride, and tetrakis[hydroxymethyl] phosphonium hydroxide are also representative of organophosphorus compounds which are suitable for use.

Examples of particular organic antimony compounds which may be used are triphenylantimony (triphenylstibine), diphenylantimony, trichloroantimony, tribromoantimony, and antimony salts of carboxylic acids, such as antimony tricaproate.

Suitable organic tin compounds include tin salts of carboxylic acids, e.g. tin octoate, tin oleate, and the various tin acrylates.

Suitable halogenated alcohols include bis[2,3-dibromopropyl] pentaerythritol, the polychlorobutanediols, and 2,3-dibromopropanol.

Examples of particular halogenated esters which may be used are Diels-Alder adducts (essentially equimolar) of alpha-beta unsaturated carboxylic acids (e.g. acrylic, methacrylic, and crotonic acid) with hexachlorocyclopentadiene.

Exemplary halogenated organic acids are chlorendic acid (hexachloroendomethylenetetrahydrophthalic acid) which may be conveniently formed by the hydrolysis of chlorendic anhydride, and tetrabromophthalic acid.

Examples of halogenated organic anhydrides which may be used are chlorendic anhydride (i.e. the Diels-Alder adduct of maleic anhydride with hexachlorocyclopentadiene), and tetrabromophthalic anhydride available commercially under the designation "Firemaster PHT4" from the Michigan Chemical Corporation.

Suitable halogenated phenolic compounds include pentachlorophenol, pentabromophenol, and halogenated compounds of bisphenol A (i.e. para, para'-isopropylidenediphenol), such as tetrabromobisphenol A (i.e. 4,4'-isopropylidenebis[2,6-dibromophenol]) available commercially under the designation "Firemaster BP4A" from the Michigan Chemical Corporation.

Examples of halogenated aliphatic hydrocarbons are the chlorinated higher paraffins, e.g. chlorinated paraffins having at least six carbon atoms per molecule. Such chlorinated hydrocarbons commonly contain about 10 to 30 or more carbon atoms per molecule and are mainly saturated straight chain hydrocarbons which range from viscous liquids to solids at room temperature. Such chlorinated paraffins are well known in the art and may contain various degrees of chlorination which generally range up to about 70 per cent chlorine by weight, e.g. about 40 to about 70 per cent chlorine by weight. Chlorinated paraffins are available commercially under the designation "Unichlor" (e.g. "Unichlor 40," "Unichlor 50," and "Unichlor 70") from the Neville Chemical Company, and "Chlorowax" from the Diamond Alkali Co. Additionally, suitable halogenated aliphatic hydrocarbons may possess a cyclic structure and include perchloropentacyclodecane, hexabromocyclododecane and hexabromododecatriene.

Suitable halogenated aromatic hydrocarbons include pentabromobenzene, pentabromotoluene, and pentachlorotoluene.

Exemplary halogenated aromatic ethers are pentabromodiphenylether, pentachlorodiphenylether, and dibromophenylether.

The silicone oils contemplated for use in the process of the present invention are water-insoluble, substantially non-volatile, liquid polysiloxanes, and any of the commonly known compositions of this type may be employed. Polysiloxanes wherein the organic radical is a low molecular weight aliphatic group such as methyl or ethyl, or wherein a high percentage of low molecular weight aliphatic groups are present, are the types most widely available and have the lowest cost, and are for this reason preferred. Examples of particular silicone oils which may be used are the polymethyl siloxanes having a viscosity of over 50 centistokes at 25°C. (Dow Corning DC-200 series) and polymethyl phenyl siloxanes of medium aromaticity (Dow Corning DC-550 silicone oil). Another commercially available material is known as "General Electric Silicone Oil No. 9981." The silicone oils are well understood in the art, being described, for instance, in chapter 4 of "Chemistry of the Silicones" by Eugene G. Rochow, 1st. Ed., 1946, and further described in chapters 5 and 6 of the 2nd edition of this book, published in 1951. The alkyl, aryl, and alkyl-aryl silicones mentioned as oils in these chapters are suitable for use according to the present invention.

Mixtures of the foregoing organic protective agents may be utilized to impregnate the preoxidized acrylic fibrous material. One may also optionally employ an additive in conjunction with the protective agent which enhances the operation of the protective agent. For example, bibenzyl (1,2-diphenylethane) has been found to exhibit a synergistic influence.

The mechanism whereby the organic protective agent renders the preoxidized acrylic fibrous material capable of withstanding the highly elevated temperature of the reducing flame (described in detail hereafter) is considered complex and incapable of simple explanation. The result obtained is considered surprising in view of the fact that the organic compounds utilized are themselves not generally recognized to be capable of enduring the temperature of the reducing flame. For instance, it is difficult to envision how the organic protective agents perform their function since these agents are observed substantially to volatilize at the high temperature of the reducing flame. While some of the organic protective agents have been utilized as flame retardants in the past they have been generally considered to have no flame retardant activity above about 500°C. Conversely, well known inorganic flame retardants, such as boric acid, which have in the past been suggested as high temperature flame retardants do not provide the protection required for successful graphitization of a preoxidized acrylic fibrous material in the reducing flame.

If the organic protective agent is a non-viscous liquid, the fibrous material may be simply contacted with the same. Most commonly however, the organic protective agent is a viscous liquid or solid. When the organic protective agent is a viscous liquid or solid, it is dissolved in a suitable solvent or carrier in order to facilitate impregnation of the fibrous material. The specific solvent selected is dictated by the solubility characteristics of the organic protective agent as will be apparent to those skilled in the art and is relatively volatile. For safety considerations it is recommended that solvents be employed which possess a relatively high self-ignition point, and which are accordingly not highly flammable.

In a preferred embodiment of the process the preoxidized acrylic fibrous material is impregnated by immersion in a liquid comprising the organic protective agent. For instance, the fibrous material while present on a mandrel, bobbin, or other support may be placed in the liquid, or a continuous length of the material may be continuously passed through the liquid. Alternatively, the liquid may be sprayed or padded upon the fibrous material; however, superior impregnation is generally achieved through immersion and is accordingly

recommended. The temperature of the liquid at the time of impregnation is not critical and may conveniently be room temperature. A highly volatile non-viscous halogenated hydrocarbon solvent may be selected to dissolve many of the organic protective agents. For instance, highly halogenated hydrocarbons such as carbon tetrachloride, perchloroethylene, tetrachloroethane, tetrabromomethane, dibromoethane, and trichloroethylene are preferred. A particularly preferred solvent is trichloroethylene. Organic protective agents such as tetrakis[[hydroxymethyl] phosphonium chloride may be applied from water solutions. The concentration of the organic protective agent in a solvent required to achieve adequate loading of the fiber within a brief period of immersion (e.g. 5 seconds) is not highly critical. For instance, concentrations of the organic protective agents in solvents generally may conveniently range from about 0.5 to 25 per cent by weight based upon the weight of the solvent (preferably about 1 to 10 per cent by weight based upon the weight of the solvent). Higher concentrations tend to yield no commensurate advantage.

The residence time during which the preoxidized acrylic fibrous material is immersed in a solution comprising the preoxidized acrylic fibrous material is somewhat dependent upon the form assumed by the material while immersed. If the fibrous material is present as a package, a longer residence time will be required for the material to be impregnated throughout. For instance, residence times in batch operations for the impregnation step may range as high as 5 minutes or more depending upon the thickness of the package. In a continuous operation in which a continuous length of the preoxidized acrylic fibrous material is continuously passed through the solution comprising the organic protective agent, the residence time conveniently may be from about 5 to 25 seconds, since adequate impregnation and coating of the fibrous material is not dependent upon extended soaking.

It is not essential that the preoxidized acrylic fibrous material be dried prior to its passage through the reducing flame. In fact, in a preferred embodiment of the process the fibrous material is continuously passed through the impregnation zone and then directly to the reducing flame for graphitization.

A highly preferred reducing flame for use in the process is that resulting from an acetylene and oxygen mixture. With this reducing flame, the graphitizing step can be conducted in an open atmosphere. A further advantage of the acetylene-oxygen reducing flame is that it has a fairly constant high temperature which is independent, within limits, of the fuel-oxidant ratio. A carbon monoxide-oxygen flame also yields good results in an open atmosphere, although it is, of course, essential to provide adequate safety provisions for the operator under such conditions. Hydrocarbon fuels, such as propane and butane, may be selected but the process does not proceed as smoothly as with acetylene or with carbon monoxide. However, in the presence of an inert blanketing gas, e.g. nitrogen, or argon, comparable stability may be achieved with hydrocarbon fuels.

Molecular oxygen can be replaced in the fuel-oxidant mixture by a gaseous oxidant such as nitrous oxide although generally it is not advantageous to do so because of the convenience and ready availability of oxygen. Fuel-oxidant combinations can also be employed to produce the reducing flame which do not contain a hydrocarbon fuel, such as a carbon monoxide-hydrogen mixture and a hydrogen-chlorine mixture. Non-conventional flame sources, such as augmented flames (cf. B. Karlovitz, International Science of Technology, June, 1962, pp. 36-41); recombination flames, such as the atomic hydrogen torch (cf. I. Langmuir, Industrial and Engineering Chemistry, June, 1927, pp. 667-674); plasma torches; and the like; can also be employed to provide high temperatures. The temperature should not be so high, however, as to destroy the fibrous configuration.

The fuel to oxidant ratio generally is a significant parameter in the present process. The graphitizing treatment is best car-

ried out in a luminous flame obtained by keeping the amount of oxygen in the fuel mixture below the stoichiometric amount which is required to burn the fuel completely to carbon dioxide. Oxidation reactions within the flame are essentially limited to the combustible gas mixture, and the fibrous material traveling through the flame is exposed to an essentially reducing environment. The fibrous material can be destroyed by oxidation if the oxidant-fuel ratio is too high. The luminosity of the flame is believed to be caused by ionized carbon fragments in the flame resulting from incomplete combustion of the fuel. More pyrolytic carbon will be deposited at higher oxygen to fuel ratios than at lower ratios. For certain applications a deposit of pyrolytic graphite is desirable since it increases the high temperature stability of the resulting graphitic product. For other applications such a deposit is undesirable, e.g., where high adhesion to a matrix is desired. Hence, the flexibility of processing conditions allows for the production of a variety of graphite product types. If desired, a surface protective layer of pyrolytic graphite alternatively can be formed in a separate step in which the fibrous material is heated to a high temperature in a controlled environment containing hydrocarbon vapors.

In the context of this specification, temperatures in the flame zone refer to the temperature of the fibrous material as measured by an infra-red radiation thermometer and not to a theoretical reducing flame temperature under adiabatic conditions, i.e. without withdrawal of heat by immersing a body into the reducing flame. The temperature of the fibrous material in the flame is generally significantly lower than the theoretical reducing flame temperature.

For example, the theoretical flame temperature of an oxygen-acetylene reducing flame is about 3,100° C. An upper limit of about 2,500° C. for the fiber temperature of a yarn undergoing treatment is generally sufficient and safe.

The impregnated fibrous material is passed through the reducing flame at a fast enough rate to avoid breaking. As the temperature of the reducing flame is increased, the minimum rate at which breakage is avoided also increases. This minimum speed can be determined for any given combination of impregnated fibrous material and specific reducing flame. The longer the residence time, the greater the extent of graphitization. Thermal degradation with graphite formation occurs within the reducing flame to the substantial exclusion of oxidative degradation. Optimum conditions are reached at the point where the loss of the fiber mass is lowest and the conversion of the remainder of the fibrous material to graphitic carbon is the highest. The two effects can be balanced favorably by adjusting the residence time and the fiber temperature. Subject to the nature of the reducing flame and other factors, residence times of about 2 to 24 seconds, and preferably about 6 to 17 seconds are generally suitable. An exemplary set of optimum conditions is a yarn temperature of 2,300° C. with a residence time of about 15 seconds.

The necessary apparatus for graphitization according to the present process is simple and should be so arranged that the fibrous material is exposed to a minimum of frictional contacts. A convenient arrangement is to continuously feed an impregnated yarn from a rotating-reciprocating bobbin through the reducing flame to an identically functioning take-up mechanism. Starting at the correct reciprocating position on the bobbin, the yarn is unwound without traverse movement and analogously rewound at the take-up side. Hence, random yarn motions are minimized. Further positioning of the yarn in the reducing flame can be accomplished with minimal action by two cylindrically shaped guides located before and after the reducing flame source. Feed and take-up bobbins can be driven by, for example, solid-state controlled DC motors with r.p.m. generator/indicators. When an inert atmosphere is desired, a cruciform glass vessel fitted with cooling plates and a passage opening for the yarn can be employed. Before entering the burner module, the yarn may be put under constant tension as, for example, by passing it over a rubber-capped electro-magnetic clutch and a skewed roll. The

latter separates individual yarn loops around the clutch and prevents abrasion by yarn to yarn contact.

The geometry of the burner is also a factor in maximizing the effectiveness of the graphitization of the present invention.

- 5 Two impinging flames originating from two standard conical tips significantly raise the temperature of the fibrous material passing therethrough. A particularly preferred embodiment of this technique is the impingement of the two reducing flames on the tips of their inner cones at an angle of 45°. However, 10 the addition of more than two orifices does not have a beneficial effect. A series of burners such as to form a continuous reducing flame zone of increased lateral dimension may permit increased processing speeds or the processing of larger fibrous assemblages. Since residence time in the reducing flame is a major parameter, processing speed is significantly related to the length of the flame zone. Surrounding the conical tip with a cylindrical or globular reflector, constructed from polished stainless steel sheets, for example, also significantly raises the yarn temperature.

15 The volume flow of the fuel and oxidant through the burner should be as high as possible, consistent with good reducing flame stability, in order to maximize the moduli of the fibers.

Tension during reducing flame treatment is recommended

- 20 for the achievement of optimum properties as it prevents the tendency of the fibrous material to shrink. Shrinkage usually leads to relaxation of ordered structures and, thereby, causes a lowering of physical properties. Preservation of orientation and/or an increase in orientation, depending upon the magnitude of tension applied, increases both the Young's modulus and the tensile strength. The tension applied should be at least sufficient to avoid visible sagging. Beyond the optimum tension the fibrous material may be damaged by still higher tensions.

- 25 30 35 Graphite fibers produced according to the present process may possess relatively uniform properties. Although I do not wish to be limited by the theory of this improvement, it appears to be due to two factors: (1) the flame healing of flaws by ionized carbon fragments in a luminous reducing flame, and (2) the reduced mechanical wear of the fibrous material in the reducing flame.

40 The following examples are given as specific illustrations of the invention. It should be understood, however, that the invention is not limited to the specific embodiments which follow.

#### EXAMPLE 1

The data in Table I illustrate the results obtainable to an embodiment of the invention wherein a tris[2,3-dibromopropyl] phosphate organic protective agent is applied on a batch basis and an acetylene-oxygen reducing flame source is utilized to form a graphite yarn from a preoxidized acrylonitrile homopolymer yarn.

- 55 A 760 continuous filament acrylonitrile homopolymer yarn was preoxidized in air at about 270° C. in a Lindberg muffle furnace on a continuous basis in accordance with the teachings of U.S. Ser. No. 749,957, filed on Aug. 5, 1968 in my name, which is assigned to the same assignee as the instant invention, and is herein incorporated by reference. The acrylonitrile homopolymer yarn had a twist of about 0.5 tpi. The preoxidized yarn exhibited a bound oxygen content of about 8 per cent by weight as determined by the Unterzaucher analysis and a carbon content of about 62 per cent by weight. The preoxidized yarn was non-burning when subjected to an ordinary match flame, but was incapable of withstanding a reducing flame when heated for two seconds at a fiber temperature of 1,900° C. The preoxidized yarn exhibited an amorphous X-ray diffraction pattern, and had a denier of 1.93, a single filament tenacity of 1.89 grams/denier, a single filament Young's modulus of about 100 grams/denier, and an elongation of 7.3 per cent.

60 65 70 75 A 10 per cent by weight solution of tris[2,3-dibromopropyl] phosphate in trichloroethylene based upon the weight of the

solvent was prepared and present at room temperature (i.e. about 23° C.). The preoxidized acrylonitrile homopolymer yarn while wound on a bobbin was immersed in the solution for about 1 1/2 minutes in order to thoroughly impregnate the same with the organic protective agent.

The yarn was next continuously graphitized without drying the same. In the manner described above the yarn was passed in the open atmosphere through an acetylene-oxygen reducing flame in which the volume ratio of the gases was 1:1. The total flow rate was 1,500 ml./min. and a "National Blow Torch", Tip AO-3 was employed. The acetylene-oxygen reducing flame imparted a fiber temperature of about 2,200° C. to the yarn. The tension applied to the yarn was varied as indicated and no visible sagging of the yarn was apparent in any of the runs. The following Table I summarizes the properties (single filament breaks) of the resulting graphite yarn as a function of the residence time of the yarn in the reducing flame.

TABLE I

| Residence time in reducing flame (seconds) | Tension (grams) | Denier | Tenacity (grams/denier) | Young's modulus (grams/denier) |
|--------------------------------------------|-----------------|--------|-------------------------|--------------------------------|
| 8                                          | 0               | 0.72   | 6.0                     | 1,018                          |
| 6                                          | 0               | 0.56   | 6.7                     | 1,235                          |
| 4                                          | 0               | 0.69   | 3.9                     | 947                            |
| 4                                          | 50              | 0.69   | 3.3                     | 1,057                          |
| 4                                          | 80              | 0.54   | 5.4                     | 1,233                          |

## EXAMPLE 2

The data in Table II illustrate the results obtainable in an embodiment of the invention wherein a tris[2,3-dibromopropyl] phosphate protective agent is applied on a continuous basis to the preoxidized acrylic fibrous material from solutions of the agent of various concentrations in trichloroethylene.

The preoxidized acrylic fibrous material identified in Example 1 was continuously passed through the solutions containing the organic protective agent for a residence time of about 8 seconds, and subsequently flame graphitized according to the procedure of Example 1 without first drying the same. In each instance the tension applied to the yarn while present in the reducing flame was sufficient to prevent visible sagging. The following Table II summarizes the properties (single filament breaks) of the resulting graphite yarn as a function of the concentration of the protective agent in the trichloroethylene solvent in weight per cent based upon the weight of the solvent.

TABLE II

| Concentration of protective agent in solvent (percent) | Residence time in reducing flame (seconds) | Tension (grams) | Denier | Tenacity (grams/denier) | Young's modulus (grams/denier) |
|--------------------------------------------------------|--------------------------------------------|-----------------|--------|-------------------------|--------------------------------|
| 7.5                                                    | 8                                          | 0               | 0.71   | 5.5                     | 1,125                          |
| 10                                                     | 8                                          | 0               | 0.86   | 5.6                     | 1,303                          |
| 15                                                     | 8                                          | 0               | 0.84   | 5.1                     | 1,107                          |

## EXAMPLE 3

Example 2 was repeated with the exception that the trichloroethylene solution of organic protective agent comprised a combination of 10 per cent tris[2,3-dibromopropyl] phosphate, 1 per cent bibenzyl, and 1 per cent silicone oil, and the preoxidized yarn was present in the same for a residence time of about 6 seconds. The concentrations are expressed in weight per cent based on the weight of the solvent. The silicone oil was a polymethyl siloxane having a viscosity in excess of 50 centistokes at 25° C. and available commercially from the Dow Corning Corporation under the designation "DC-200."

Summarized below are the graphitization conditions and the properties (single filament breaks) of the resulting graphite yarn.

|   |                                            |       |
|---|--------------------------------------------|-------|
| 5 | Residence time in reducing flame (seconds) | 6     |
|   | Tension                                    | 0     |
|   | Denier                                     | 0.64  |
|   | Tenacity (grams/denier)                    | 4.2   |
|   | Young's modulus (grams/denier)             | 1,383 |

## EXAMPLE 4

Example 2 was repeated with the exception that the organic protective agent was solely the silicone oil described in Example 3 which was applied from a 10 per cent by weight solution in trichloroethylene based on the weight of the solvent.

Summarized below are the graphitization conditions and the properties (single filament breaks) of the resulting graphite yarn.

|    |                                            |      |
|----|--------------------------------------------|------|
| 15 | Residence time in reducing flame (seconds) | 8    |
|    | Tension                                    | 0    |
|    | Denier                                     | 0.70 |
| 20 | Tenacity (grams/denier)                    | 1.75 |
|    | Young's modulus (grams/denier)             | 852  |

## EXAMPLE 5

25 Example 2 was repeated with the exception that the organic protective agent was a 10 per cent by weight solution of tricresyl phosphate in trichloroethylene based upon the weight of the solvent. The residence time for the preoxidized yarn in the solution was about six seconds.

30 Summarized below are the graphitization conditions and the properties (single filament breaks) of the resulting graphite yarn.

|    |                                            |      |
|----|--------------------------------------------|------|
| 35 | Residence time in reducing flame (seconds) | 6    |
|    | Tension                                    | 0    |
|    | Denier                                     | 0.72 |
|    | Tenacity (grams/denier)                    | 3.45 |
|    | Young's modulus (grams/denier)             | 976  |

## EXAMPLE 6

Example 2 was repeated with the exception that the organic protective agent comprised a combination 1 per cent by weight of the silicone oil described in Example 3, and 1 per cent by weight of bibenzyl in trichloroethylene based upon the weight of the solvent.

Summarized below are the graphitization conditions and the properties (single filament breaks) of the resulting graphite yarn.

|    |                                            |       |
|----|--------------------------------------------|-------|
| 60 | Residence time in reducing flame (seconds) | 6     |
|    | Tension                                    | 0     |
|    | Denier                                     | 0.62  |
|    | Tenacity (grams/denier)                    | 3.0   |
|    | Young's modulus (grams/denier)             | 1,096 |

## EXAMPLE 7

Example 2 is repeated utilizing a different reducing flame, i.e. a mixture of oxygen and propane, to produce graphite yarn. The impregnated preoxidized acrylonitrile homopolymer yarn is passed through an oxygen-propane reducing flame in which the volume ratio of oxygen to propane is 3.5:1, and a fiber temperature of approximately 2,000° C. is imparted to the yarn. The apparatus includes a cruciform glass vessel with provision for maintaining a nitrogen atmosphere therein, and is fitted with cooling plates

and passage openings for the fiber. A surface-mix propane-oxygen burner is mounted within the vessel.

#### EXAMPLE 8

Example 2 is repeated with the exception that the organic protective agent is present as a 7.5 per cent by weight solution based upon the weight of the solvent of triphenylantimony in trichloroethylene.

#### EXAMPLE 9

Example 2 is repeated with the exception that the organic protective agent is present as a 5 per cent by weight solution based upon the weight of the solvent of antimony tricaproate in trichloroethylene.

#### EXAMPLE 10

Example 2 is repeated with the exception that the organic protective agent is present as a 7.5 per cent by weight solution based upon the weight of the solvent of tin octoate in trichloroethylene.

#### EXAMPLE 11

Example 2 is repeated with the exception that the organic protective agent is present as a 10 per cent by weight solution based upon the weight of the solvent of bis[2,3-dibromopropyl] pentaerythritol in trichloroethylene.

#### EXAMPLE 12

Example 2 is repeated with the exception that the organic protective agent is present as a 10 per cent by weight solution based upon the weight of the solvent of an equimolar Diels-Alder adduct of methacrylic acid with hexachlorocyclopentadiene in which trichloroethylene serves as solvent.

#### EXAMPLE 13

Example 2 is repeated with the exception that the organic protective agent is present as a 5 per cent by weight solution based upon the weight of the solvent of chlorendic acid (hexachloroendomethylenetetrahydrophthalic acid) in trichloroethylene.

#### EXAMPLE 14

Example 2 is repeated with the exception that the organic protective agent is a 7.5 per cent by weight solution based upon the weight of the solvent of tetrabromophthalic anhydride in trichloroethylene.

#### EXAMPLE 15

Example 2 is repeated with the exception that the organic protective agent is a 10 per cent by weight solution based upon the weight of the solvent of pentachlorophenol in trichloroethylene.

#### EXAMPLE 16

Example 2 is repeated with the exception that the organic protective agent is a 10 per cent by weight solution based upon the weight of the solvent of a mixture of chlorinated higher paraffins (available commercially under the designation "Unichlor 50" from the Neville Chemical Company) in carbon tetrachloride.

#### EXAMPLE 17

Example 2 is repeated with the exception that the organic protective agent is a 5 per cent by weight solution based upon the weight of the solvent of hexabromocyclododecane in trichloroethylene.

#### EXAMPLE 18

Example 2 is repeated with the exception that the organic protective agent is a 5 per cent by weight solution based upon the weight of the solvent of pentabromotoluene in trichloroethylene.

In a control experiment in which the preoxidized acrylonitrile homopolymer yarn was impregnated with a 4 per cent by weight aqueous solution of boric acid based upon the weight of the solvent the yarn immediately broke upon subjection of the reducing flame.

Although the invention has been described with preferred embodiments it is to be understood that variations and modifications may be resorted to as will be apparent to those skilled in the art. Such variations and modifications are to be considered within the purview and scope of the claims appended hereto.

I claim:

1. A process for producing a predominantly graphitic fibrous material from a preoxidized acrylic fibrous material derived from a fibrous precursor consisting primarily of recurring acrylonitrile units, said preoxidized acrylic fibrous material having
  - a. a carbon content of up to about 65 per cent by weight,
  - b. a relatively amorphous X-ray diffraction pattern,
  - c. a bound oxygen content of at least about 7 per cent by weight, and
  - d. an absence of structural integrity when heated for two seconds at a fiber temperature of 1,900° C., comprising: impregnating said preoxidized acrylic fibrous material with a quantity of an organic protective agent capable of rendering said material resistant to loss of structural integrity when heated for at least two seconds at a fiber temperature of 1,900° C., and
2. A process according to claim 1 wherein said preoxidized acrylic fibrous material is derived from an acrylonitrile homopolymer.
3. A process according to claim 1 wherein said preoxidized acrylic fibrous material is derived from an acrylonitrile copolymer which contains at least about 85 mol per cent of acrylonitrile units and up to about 15 mol per cent of one or more monovinyl units copolymerized therewith.
4. A process according to claim 1 wherein said preoxidized acrylic fibrous material is impregnated with said organic protective agent by immersion in the same.
5. A process according to claim 4 wherein said preoxidized acrylic fibrous material is immersed in a solvent containing said organic protective agent dissolved therein.
6. A process according to claim 1 wherein said organic protective agent is selected from the group consisting of organic phosphorus compounds, organic antimony compounds, organic tin compounds, halogenated alcohols, halogenated esters, halogenated organic acids, halogenated organic anhydrides, halogenated phenolic compounds, halogenated aliphatic hydrocarbons, halogenated aromatic hydrocarbons, halogenated aromatic ethers, silicone oils, and mixtures of the foregoing.
7. A process according to claim 1 wherein said reducing flame is generated by a fuel-oxidant mixture.
8. A process according to claim 7 wherein said oxidant is oxygen.
9. A process according to claim 8 wherein said fuel is acetylene.
10. A process according to claim 8 wherein said fuel is propane.
11. A process according to claim 7 wherein said impregnated fibrous material is passed through the luminous portion of said reducing flame.
12. A process according to claim 7 wherein the residence time of said impregnated fibrous material in said reducing flame is from about 2 to 24 seconds.
13. A process according to claim 9 wherein the residence time of said impregnated fibrous material in said reducing flame is from about 6 to 17 seconds.

14. A process according to claim 8 wherein the ratio of oxygen to fuel is such that the amount of oxygen is less than the stoichiometric amount required to completely oxidize said fuel.

15. A process according to claim 10 wherein an inert atmosphere is provided around said reducing flame.

16. A process according to claim 1 wherein said preoxidized acrylic fibrous material is a yarn.

17. A continuous process for producing a predominantly graphitic fibrous material from a preoxidized acrylic fibrous material derived from a fibrous precursor consisting primarily of recurring acrylonitrile units, said preoxidized acrylic fibrous material having

a. a carbon content of up to about 65 per cent by weight,

b. a relatively amorphous X-ray diffraction pattern,

c. a bound oxygen content of at least about 7 per cent by weight, and

d. an absence of structural integrity when heated for two seconds at a fiber temperature of 1,900° C., comprising:

passing said preoxidized acrylic fibrous material through a zone containing an organic protective agent capable of rendering said material resistant to loss of structural integrity when heated for at least two seconds at a fiber temperature of 1,900° C. selected from the group consisting of organic phosphorus compounds, organic antimony compounds, organic tin compounds, halogenated alcohols, halogenated esters, halogenated organic acids, halogenated organic anhydrides, halogenated phenolic compounds, halogenated aliphatic hydrocarbons, halogenated aromatic hydrocarbons, halogenated aromatic ethers, silicone oils, and mixtures of the foregoing, wherein said preoxidized acrylic fibrous material is impregnated with said

15

20

25

30

organic protective agent, and passing said impregnated fibrous material through the luminous portion of a reducing flame generated by an acetylene-oxygen mixture imparting to said fibrous material a minimum temperature of at least 1,900° C. in which the ratio of oxygen to acetylene is less than the stoichiometric amount required to completely oxidize the acetylene for a residence time of about 2 to 24 seconds while said fibrous material is under a tension at least sufficient to prevent visible sagging.

18. A continuous process according to claim 17 wherein said preoxidized acrylic fibrous material is derived from an acrylonitrile homopolymer.

19. A continuous process according to claim 17 wherein said preoxidized acrylic fibrous material is derived from an acrylonitrile copolymer which contains at least about 85 mol per cent of acrylonitrile units and up to about 15 mol per cent of one or more monovinyl units copolymerized therewith.

20. A continuous process according to claim 17 wherein said preoxidized acrylic fibrous material is passed through a zone containing said organic protective agent dissolved in a solvent.

21. A continuous process according to claim 20 wherein said solvent is a halogenated hydrocarbon.

22. A continuous process according to claim 21 wherein said solvent is trichloroethylene.

23. A continuous process according to claim 17 wherein the residence for said impregnated fibrous material in said reducing flame is about 6 to 17 seconds.

24. A continuous process according to claim 17 wherein said preoxidized acrylic fibrous material is a yarn.

\* \* \* \* \*